

R. L. FOWLER.

RECLAMATION OF DISCARDED MINERAL SURFACE ROOFING.  
APPLICATION FILED NOV. 1, 1918.

1,290,959.

Patented Jan. 14, 1919.



Inventor

Robert L. Fowler;

Witnesses  
John C. Berger  
James H. Bell

by *Jolley & Pace*

Attorneys:

# UNITED STATES PATENT OFFICE.

ROBERT L. FOWLER, OF PERTH AMBOY, NEW JERSEY, ASSIGNOR TO THE BARBER ASPHALT PAVING COMPANY, OF PHILADELPHIA, PENNSYLVANIA, A CORPORATION OF WEST VIRGINIA.

## RECLAMATION OF DISCARDED MINERAL-SURFACE ROOFING.

1,290,959.

Specification of Letters Patent.

Patented Jan. 14, 1919.

Application filed November 1, 1918. Serial No. 260,760.

To all whom it may concern:

Be it known that I, ROBERT L. FOWLER, a citizen of the United States, residing in Perth Amboy, in the State of New Jersey, have invented certain new and useful Improvements in the Reclamation of Discarded Mineral-Surface Roofing, of which the following is a specification, reference being had to the accompanying drawings.

10 In the manufacture of prepared roofing with mineral or grit surface, a certain amount of so-called mill ends, or other portions, are necessarily discarded by reason of imperfection. Usually, the imperfections 15 are in the grit surface of the roofing and are due to irregularities or intermissions in the operation of applying the surfacing bitumen or the grit coating. In either case, the resulting imperfection of the final grit surface 20 spoils the appearance of the roofing, making it necessary to cut out such defective parts with corresponding loss to the manufacturers. The parts thus cut out must either be discarded as waste or else sold at less than 25 cost as seconds.

I have discovered that if the surfaces of shingles or sheet roofings, which are partially or imperfectly coated and gritted, are exposed to a suitable temperature, the bituminous crust underlying the grit may be softened and caused to flow together as a smooth coating and, in this condition, while the coating is warm and plastic, if a fresh supply of grit is distributed over the surface and pressed into it, it will adhere wherever the grit was hitherto lacking, and thus restore the sheet to its condition as first-class roofing material.

30 I have devised a simple apparatus for carrying out this process which is illustrated more or less diagrammatically in the accompanying drawing.

The apparatus consists of an endless conveyer 1, of asbestos or other suitable non-combustible, insulating material. The conveyer is driven in the direction of the arrow under the propulsion of the supporting rolls 2 and 3, running at a slow, even rate of speed. The imperfect shingles 5, are successively laid or fed to the conveyer face up-

wards and advanced through an electric heating device comprehensively indicated at 5, binding posts 6, being provided for attachment of the line conductors 7.

In practice, I have found that by subjecting the shingles to a temperature from 600° to 1000° F., for a period of two (2) to five (5) minutes, the surface layer of bitumen will become sufficiently soft and will flow sufficiently for the present purposes without injury to the remaining parts of the structure or causing the bitumen to overrun the portions of the surface already covered with the grit.

After emerging from the heating device, 65 the shingles are passed beneath a hopper 10, from which grit is cascaded as illustrated. Said hopper is provided with appropriate controlling means 11, whereby the rate of flow of the grit may be accurately regulated. 70 After this, the shingles are delivered beneath a compression roll 12, which cooperates with the driving roller 3, of the conveyer. By the latter action, the grit is firmly pressed into the fused bare spots of 75 the shingles with the result that the surface becomes uniformly coated and the product saleable as a first-class article.

The sheets are discharged from the machine, under the guidance of an inclined 80 screen 15. The surplus grit drops through the latter and is collected in a receiving trough from which it may from time to time be returned to the hopper 10.

Having thus described my invention, I 85 claim—

The process of restoring imperfectly gritted roofing material which consists in subjecting the imperfect surface to heat sufficient to soften and distribute the bituminous 90 coating; applying additional grit thereto while still soft; and pressing the grit into the softened bituminous surface.

In testimony whereof I have hereunto signed my name at Philadelphia, Pennsylvania, this twenty-first day of October, 1918.

ROBERT L. FOWLER.

Witnesses:

WILLIAM A. O'DONNELL,  
JOSEPH G. SCHUCK.